

## UNITED STATES PATENT OFFICE

1,991,886

## PRODUCTION OF COLORATIONS ON MATERIALS

George Holland Ellis, Spondon, near Derby, England, assignor to Celanese Corporation of America, a corporation of Delaware

No Drawing. Application January 25, 1933, Serial No. 653,476. In Great Britain February 10, 1932

## 3 Claims. (Cl. 8—5)

This invention relates to the production of effects on textile materials and more particularly to the production of effects on such materials made of or containing cellulose acetate or other cellulose esters.

In the production of discharge or resist effects on textile materials it is customary either to apply a ground colour to the material and then to print the coloured material with a composition containing a discharging agent or to apply the discharging composition to the material before the application of the ground colour so that colouration by the ground colour does not take place in the printed areas. Where coloured pattern effects are desired, colouring matter resistant to the discharging agent and having affinity for or capable of being fixed on the material is incorporated in the discharging composition.

In the production of pattern effects on materials comprising an organic ester of cellulose, however, it has been found that the application of a composition containing a discharging agent to the coloured material does not always give complete discharge of the ground colour as readily as is desirable. Where a deeply coloured pattern, e. g. navy blue, is to be produced, this may not be of such great importance, but where a white or delicately coloured pattern is required it is a matter of the utmost importance that the ground colour should be completely discharged in the printed areas.

It has now been found that good discharge of a ground colour on materials made of or containing cellulose esters can readily be obtained if, after colouration with the ground colour but prior to the application of the discharging composition, the material is subjected to a saponification treatment for the cellulose ester.

According to the present invention, therefore, discharge or discharge resist effects are produced on materials made of or containing cellulose esters by a process comprising a saponification of the cellulose ester portions of the materials after colouration, but before effecting the discharge.

Among saponifying agents which may be employed for the process of the present invention are caustic soda, caustic potash, sodium or potassium carbonate, sodium silicate, or trisodium phosphate. These agents may, if desired, be in aqueous or alcoholic solution. They may further be employed in conjunction with any other desired substances, such for example as swelling agents for the material. A particularly suitable saponifying agent is a 2 to 10% solution of caustic soda in a mixture of alcohol and water.

The saponifying agent may be applied by any convenient method, e. g. by padding or other method of mechanical impregnation. After application of the saponifying agent the material is preferably steamed, aged, or dried to bring about or to complete saponification to the desired extent.

The amount of saponification necessary to lead to improved discharges on cellulose acetate materials is small. For the best results, however, it has been found desirable to saponify so that there is a loss in weight of at least 5%, e. g. 10 or 15% or more. In the case of other esters an equivalent degree of saponification may be employed.

The discharge of the ground colouration may be effected with the aid of any suitable discharging agent, for example reducing discharging agents such for example as aldehyde or ketone sulphoxylates, particularly zinc formaldehyde sulphoxylate, hydrosulphites, stannous salts, such for example as stannous chloride, or oxidation discharges, e. g. chlorates or chromates. The discharge compositions may contain any other desired ingredients, e. g. swelling agents, catalysts and/or delustering or relustering agents for the cellulose ester portion of the material, such for example as alcohols, phenol, anthraquinone, hydroquinone and urea.

Where coloured pattern effects are to be produced the compositions may contain dyestuffs resistant to the discharging agent but having an affinity for or capable of being fixed on the saponified fibre, or dyestuff components or leuco compounds which may subsequently be developed or oxidized on the fibre. Thus for example where saponification has been carried out only to a small extent any of the usual dyestuffs employed in the colouration of cellulose ester materials and which are resistant to the discharging agent may be used for colouring the discharging composition. Where saponification has been carried out to a greater extent dyestuffs having an affinity for cotton may be employed for this purpose.

The discharging composition may be applied to the material in any convenient manner. Thus for example it may be applied by printing or through stencils.

As has been indicated the process of the present invention may be applied to material of any cellulose ester capable of saponification. Thus for example it may be applied to materials made of or containing cellulose acetate, cellulose formate, cellulose propionate or cellulose butyrate. It is however equally applicable to materials containing these cellulose esters in admixture with other

textile fibres, e. g. cellulose ether fibres, regenerated cellulose, cotton, wool or silk fibres. In this connection, by suitably adjusting the degree of saponification of the cellulose ester, it is possible to obtain very valuable effects on materials containing other fibres in addition to the cellulose ester. Thus for example a mixed fabric containing cellulose acetate and cotton may be cross dyed with dyestuffs having an affinity for cellulose acetate and with dyestuffs having an affinity for cotton, the cellulose acetate saponified until it acquires affinity for cotton dyestuffs, and the material then printed with a discharge composition containing a dyestuff resistant thereto and having an affinity for cotton, when a coloured pattern effect on a cross dyed ground is obtained.

The following examples illustrate the invention without being in any way limitative:—

*Example 1*

20 A woven cellulose acetate fabric dyed a red shade with 4-nitro-2-methoxybenzene-1-azo-4'-dimethylaminobenzene is saponified to an extent corresponding to a loss in weight of about 10% by cover padding with a 15% solution of sodium carbonate suitably thickened with starch thickening, and then drying and steaming for example in a Mather and Platt rapid ager. The fabric is then washed off thoroughly and dried. The 25 saponified fabric is now printed with a printing paste having the following composition:—

|                                | Parts |
|--------------------------------|-------|
| Zinc formaldehyde sulphoxylate | 25    |
| Methylated spirits             | 10    |
| Ethyl lactate                  | 10    |
| Gum arabic thickening          | 55    |
|                                | 100   |

40 The printed goods are then dried, aged for 5 to 7 minutes in a Mather and Platt ager and finally washed thoroughly and dried or subjected to any other treatments which may be desirable or requisite. An excellent white discharge print is obtained on a red ground, the discharge being more 45 complete than a discharge attained under parallel conditions on unsaponified materials.

*Example 2*

50 A woven cellulose acetate fabric dyed a red-violet shade with 2:4-dinitrobenzene-azo-4-diethylaminobenzene is padded with an 8% solution of caustic soda, squeezed with rollers which are so adjusted that the fabric retains approximately 55 80% of its weight of liquor, and passed

over heated drums to effect simultaneous drying and saponification of the goods. The degree of saponification is of the order of that corresponding to a loss in weight of 5%. The material is then printed, if desired, after washing and drying with a printing paste having the following composition:—

|                                  | Parts |
|----------------------------------|-------|
| Sodium formaldehyde sulphoxylate | 10    |
| Potassium carbonate              | 12    |
| Methylated spirit                | 10    |
| Gum thickening and water         | 68    |
|                                  | 100   |

15 The fabric is then dried, steamed in a Mather and Platt ager or in a vat steamer, washed off and dried, when an excellent white discharge is obtained on the red-violet ground. If coloured discharge effects are required, vat dyestuffs may be 20 incorporated in the above printing paste.

*Example 3*

25 A fabric consisting of equal parts of cotton and cellulose acetate, and dyed in contrasting shades with 2-nitro-4-methyl-benzene-azo-para-xylydine on the acetate, and Chlorazol Fast Blue 2BN (see page 345 of Color Index) on the cotton, is padded with a 6% solution of sodium carbonate, the conditions being such that the fabric takes up 30 100% of its own weight of liquor. It is then dried on a stenter and steamed in a Mather and Platt ager or in a vat steamer, and finally printed according to either of the discharge processes of Examples 1 or 2, steamed or aged, and washed and 35 dried, when excellent discharges are obtained on a two colour ground.

What I claim and desire to secure by Letters Patent is:—

1. In the production of discharge effects on materials made of or containing cellulose esters, saponifying the materials after colouration with a ground colour but prior to discharge of that ground colour.
2. Process according to claim 1, characterized in that the cellulose ester is cellulose acetate.
3. Process for the production of discharge effects on materials made of or containing cellulose acetate, which comprises saponifying the materials after coloration with a ground color, to such an extent that the cellulose acetate loses between 5 and 15% of its weight, and thereafter discharging the ground color.

GEORGE HOLLAND ELLIS. 55